

July 23, 1940.

J. EGGERT ET AL

2,208,754

MULTIPACK PHOTOGRAPHY

Filed Dec. 11, 1935

Fig. 1



Fig. 2



John Eggert  
Arpad von Biehler  
Gerd Heymer  
Inventors

By their Attorneys

Shutz and Joslin

## UNITED STATES PATENT OFFICE

2,208,754

## MULTIPACK PHOTOGRAPHY

John Eggert, Leipzig-Gohlis, Arpad von Biehler,  
 Dessau, and Gerd Heymer, Wolfen Kreis  
 Bitterfeld, Germany, assignors, by mesne assignments, to General Aniline & Film Corporation, New York, N. Y., a corporation of Delaware

Application December 11, 1935, Serial No. 53,872  
 In Germany December 13, 1934

## 1 Claim. (Cl. 95—2)

This invention relates to multipack photography.

One of its objects is a multipack with which sharper pictures are obtainable than hitherto usual. Further objects will be seen from the detailed specification following hereafter. Reference is made to the accompanying drawing in which Fig. 1 shows a tripack of normal film and Fig. 2 shows a lenticular bipack in accordance with the invention.

In the production of multicolor pictures by means of the usual bi- and tripacks, there is placed in front of the second and third layer, respectively, in the pack a yellow or red filter in some suitable form, for instance, as an intermediate separate film or as a colored coating on the emulsion side or the opposite side of the support, or the carrier itself may be colored. The emulsion layers behind this filter are thus sensitized for corresponding kinds of light. The light filters consisting of separate films or layers interposed in the pack have the disadvantage that the distance between the several emulsion layers is increased, so that the rear pictures produced are not so sharp as the remainder. The colored support does not present this drawback but the support cannot subsequently be decolorized and therefore renders the picture unsuitable for copying.

According to this invention there is used a fine-grained emulsion, rich in silver, which is differently sensitized for each layer, so as to produce the desired color separation, it being advantageous to damp the specific blue sensitivity of the emulsion by the known method of directly dyeing the emulsion with a screening dye, for instance, a yellow dyestuff. The grain of the emulsion layers in the multipack should not exceed a mean value of  $1\mu$  diameter and the ratio of silver to gelatin should be at least 1 part of silver on 1.5 parts of gelatin the parts being by weight.

The material made by the invention is therefore without any colored layer between the emulsion layers sensitized for different spectral ranges; this is a substantial simplification in the manufacture and leads to improved sharpness in the rear picture. The invention is ap-

plicable for all tripack arrangements; advantageously it is combined with the invention described in U. S. patent application Serial No. 48,337, which deals with the production of pictorial swollen reliefs from thin, extremely highly hardened layers of emulsion. In the tripack according to this invention the blue sensitive film is preferably arranged next the source of light, whereas the films sensitive to green and red may follow in optional manner.

The invention is also useful in the production of the two-pack lenticular film described in U. S. Patent No. 1,968,944. In this case the resolution into the fundamental colors is produced in part by the filter and screen and in part by a spectral method with the aid of differently colored and sensitized layers. The use of finely-grained layers rich in silver makes it unnecessary in this case to introduce a red filter layer as has hitherto been usual, whereby, moreover, the assistance of the two-zone filter arrangement in front of the objective still favours the sharp separation between the red and green details. In this manner there is obtained a separation of the fundamental colors which is better than when filters or sensitizers are used alone.

Fig. 1 of the accompanying drawing shows a tripack consisting of three normal films, 1, 2 and 3. The front film 1 is sensitive to blue, the middle film 2 is sensitive to green and the back film is sensitive to red. Fig. 2 shows a lenticular bipack in which the lenticular front film 4 is sensitive to blue and green, and the smooth back film 2 is sensitive to red.

What we claim is:

A combination of a multipack consisting of a lenticular film in contact with a smooth film and not being separated by any filter layers, each film consisting of a support coated with a silver halide gelatin emulsion layer having a grain size not exceeding a mean value of  $1\mu$  diameter, the ratio of silver to gelatin being at least 1 part of silver on 1.5 parts of gelatin, the parts being by weight, and the two emulsion layers being sensitized to different spectral regions.

JOHN EGGERT.

ARPAD VON BIEHLER.

GERD HEYMER.